

## UNITED STATES PATENT OFFICE.

JOSEPH C. STONE, OF BELMONT, MASSACHUSETTS.

## ALLOY.

No Drawing.

Application filed April 4, 1922. Serial No. 549,570.

To all whom it may concern:

Be it known that I, JOSEPH C. STONE, a citizen of the United States, residing at Belmont, in the county of Middlesex and State 5 of Massachusetts, have invented certain new and useful Improvements in an Alloy, of which the following is a specification.

This invention relates to alloys from which metal parts may be made that are to 10 be subjected to the action of acids, or are to be used where they are likely to come in contact with materials or solutions that would corrode metals of the usual kinds. The invention is concerned particularly with 15 the provision of an alloy from which the pipe fittings and metal parts that hold or conduct milk in dairies can be made. It is very important that milk shall not be contaminated by its contact with the pipe fittings or containers, and consequently it is 20 essential that the acids of the milk shall not attack these metal parts. Similar problems also exist in numerous other industries, as for instance, in the paper and pulp industry, 25 where pipe fittings and valves are subjected to the action of solutions containing a substantial percentage of sulphuric acid.

I have discovered that a very superior alloy can be made of copper, nickel, lead and 30 tin in substantially the following proportions:—For castings, such for instance, as pipe fittings for dairies, I prefer a composition consisting of approximately

35      73%-----copper  
      17½%-----nickel  
      3½%-----tin  
      6%-----lead

For sheets, or parts that are to be rolled, I 40 prefer to vary the formula slightly and to use about

45      76%-----copper  
      20%-----nickel  
      2½%-----tin  
      1½%-----lead

For valves and other parts that are to be used in the handling of the sulphuric acid

solutions dealt with in pulp and paper making, I prefer a composition consisting of 50 substantially

|     |       |        |    |
|-----|-------|--------|----|
| 70% | ----- | copper | 55 |
| 20% | ----- | nickel |    |
| 4%  | ----- | lead   |    |
| 6%  | ----- | tin    |    |

It will be understood, of course, that the percentages of the constituents may be varied within reasonable limits. I prefer to use materials that are as pure as possible 60 and that are particularly free from aluminum, zinc, or iron, although a trace of any one of these ingredients is, for most purposes, not a serious factor.

The alloy is made by melting the constituents together in the usual manner, preferably with the aid of a flux, such as zinc or carbon free manganese. The percentage of such a flux used can be very small, say about 1%, so that it will be completely oxidized 70 during the compounding process, and the product, therefore, will not contain any, or at most only a trace, of the material used as a flux.

An alloy of the composition above described has proved very satisfactory indeed for the particular purposes above mentioned. It has been used with especial satisfaction in dairies, pulp and paper mills, for the metal parts of soda fountains, coffee urns, and the 80 like. It effectively resists the action of acids, such as those found in milk, pulp liquor, and the like, it machines readily, and presents a pleasing appearance when properly finished. In addition this alloy finds 85 many important uses in the jewelry trade, in marine work, and in locations where the metal parts are exposed to the weather or to the action of corrosive agents. The alloy in sheet form has considerable resiliency and is 90 a valuable material from which to make springs that must be subjected to the action of corrosive agents.

Having thus described my invention, what I desire to claim as new is:

1. An alloy of the character described con-

sisting essentially of the following constituents in substantially the proportions named:

5      Copper-----70 to 76%  
 Nickel-----17 to 20%  
 Lead-----1½ to 6%  
 Tin-----2½ to 5%

2. An alloy of the character described

consisting essentially of the following constituents in approximately the proportions named:

Copper-----73 %  
 Nickel-----17½ %  
 Tin-----3½ %  
 Lead-----6 %

JOSEPH C. STONE.